

June 15, 1965

C. C. BARD ET AL

3,189,452

COLOR-FORMING PHOTOGRAPHIC PROCESS UTILIZING A  
BLEACH-FIX FOLLOWED BY A BLEACH  
Filed Dec. 5, 1961



Fig. 1



Fig. 2

Charleton C. Bard  
George P. Varlan  
INVENTORS

BY *R. Frank Smith*  
*Lawrence B. Willis*

ATTORNEYS

1

3,189,452  
COLOR-FORMING PHOTOGRAPHIC PROCESS  
UTILIZING A BLEACH-FIX FOLLOWED BY  
A BLEACHCharleton C. Bard and George P. Varlan, Rochester, N.Y.,  
assignors to Eastman Kodak Company, Rochester, N.Y.,  
a corporation of New JerseyFiled Dec. 5, 1961, Ser. No. 157,096  
4 Claims. (Cl. 96—55)

The present invention relates to photography and particularly to the processing of color photographic materials. Still more particularly, the invention relates to a shortened method for the processing of coupler-incorporating, color-forming photographic films and prints.

In the usual method for processing of exposed multilayer coupler-incorporating, color-forming photographic materials, the color developer bath is usually followed by consecutive baths comprising a fix, a bleach, and a fix again with an intervening wash step between each of the baths indicated. As is well known, the fix bath is employed to remove the undeveloped silver halide from the developed emulsion layers while the bleach bath is employed to oxidize the metallic silver formed by development to silver halide. The second fix is normally employed to remove the silver halide formed by the previous bleaching step so that the emulsion layers are cleared of residual silver and silver halide. This leaves essentially a colored image of cyan, magenta, and yellow dye densities as formed at the time of development by coupling of the incorporated couplers with oxidation products of a primary aromatic amino developing agent contained in the color developer bath.

It has been of interest for some time to shorten the time required for processing of color-forming photographic materials. The present invention has quite unexpectedly found a shortened method for the processing of certain color-forming photographic materials without sacrifice in image quality and which is adapted for use in the processing of photographic materials of a high silver content. By high silver content in the present specification, we mean materials having a silver content of 200 mg. per square foot or higher. The image quality obtained according to the present invention is illustrated in the accompanying drawing in which:

FIG. 1 shows the colored image densities obtained in a standard photographic process.

FIG. 2 shows the colored image densities obtained using the present shortened process.

Accordingly, it is an object of the present invention to provide a novel shortened process for the processing of color-forming photographic materials. A second object is to provide processing baths for use in said shortened process. Other objects will become apparent from a reading of the specification and appended claims.

These objects are accomplished by treating an exposed color-forming photographic material of the invention, after color development and washing, with a combined bleaching and fixing solution followed by a separate bleaching solution. According to the invention, an intervening wash between the treating baths of the invention is not required. After the bleaching bath of the present process, the photographic material can be washed and then treated with a conventional buffer bath, if desired, as normally employed in the art.

Photographic materials of the type processed according to the present invention comprise materials having

2

color-forming couplers contained in respective layers of a multilayer photographic element. Materials of this type have been described in a number of U.S. and foreign patents, for example, in U.S. Patents 2,322,027, June 15, 1943; 2,407,210, September 3, 1946; 2,474,293, June 28, 1949; 2,640,776, June 2, 1953; and 2,956,876, October 18, 1960. Color films of the invention include the so-called negative-positive type materials as well as reversal materials. The photographic multilayer color materials of the invention comprise elements having usually three selectively sensitive emulsion layers coated on one side of a photographic support. Sensitive layers of the elements of the present invention contain color-forming couplers to form the complementary dye to which a particular layer is sensitive. In sensitive materials of this type, the uppermost layer is generally blue-sensitive and normally incorporates a yellow-forming coupler. The next layer generally comprises a filter layer which is yellow in color and blue absorbing and being placed under the top layer absorbs most of the blue light thus preventing unwanted blue exposure below the filter layer. The next layer is generally green-sensitive and usually incorporates a magenta-dye forming coupler. The emulsion layer adjacent to the support is generally red-sensitive and according to the present invention normally contains a cyan-dye forming coupler. Sometimes multilayer photographic elements as used in the present invention contain additional silver halide emulsion layers or other interlayers for specialized purposes. In photographic print materials, frequently the yellow filter layer is omitted and the arrangement of silver halide emulsion layers may be changed for the purpose of obtaining more accurate recording of the color negative.

In accordance with the present invention, the combined bleaching and fixing solution can be prepared by combining a number of silver bleaching agents and silver halide fixing agents. For example, where freshly prepared combined solutions can be employed, a suitable bleaching agent can comprise an alkali metal dichromate (e.g., sodium dichromate, and potassium dichromate), an alkali metal ferricyanide (e.g., potassium ferricyanide, and sodium ferricyanide), ferricyanide-bromide, permanganate (e.g., potassium permanganate), quinone, and the like. Such bleaching agents can be combined in freshly prepared solutions with such fixing agents as alkali metal thiocyanates (e.g., sodium thiocyanate and potassium thiocyanate), ammonium thiocyanate, alkali metal thiosulfate (e.g., sodium thiosulfate and potassium thiosulfate), ammonium thiosulfate, thioureas, and alkali metal selenocyanates (e.g., sodium selenocyanate and potassium selenocyanate). Combined baths of this type, however, are stable over a very short period of time; and, consequently, optimum results can be obtained using fresh solutions only. Some improvement in stability in such baths can be obtained by the addition to the bath of a thickening agent which results in the formation of a viscous solution. Such viscous solutions can be applied as a surface layer on the photographic material to be processed. Suitable thickening agents for this purpose include a wide variety of materials, such as carboxymethylcellulose, ethylcellulose, gelatin, polyvinyl alcohol, colloidion, polyvinyl acetals, cellulose esters, and the like.

More stable combined bleaching and fixing solutions comprise, for example, a ferric chloride solution containing a sequestering agent such as ethylene diamine tetraacetic acid tetrasodium salt, and a fixing agent such as sodium thiosulfate. Other combined solutions of the

more stable variety employ a sulfur-containing dibasic acid such as ethylene-bis-thioglycolic acid as the stabilizing silver halide solvent. Solutions of this latter type have been described in P. M. Mader, U.S. Patent 2,748,000, issued May 29, 1956.

Other sequestering agents can be employed in combined solutions of the invention, for example, 1,3-diamino-2-propanol tetraacetic acid. Other suitable sequestering agents have been disclosed in "Organic Sequestering Agents," S. Chaberek and A. E. Martell, published 1959, by John A. Wiley and Sons.

The separate bleaching solution for use in the present invention can be prepared by dissolving an appropriate amount of a silver bleaching agent of the type mentioned above in water. Such bleaching agents are normally sufficiently water soluble to allow an appropriate concentration of the bleaching agent in an aqueous bath. Such solutions can also contain other ingredients as borax, sodium bromide, copper chloride, etc., as is well known in the art. Suitable processing baths of the invention have been described in the prior art in a number of U.S. and foreign patents and publications. A number of such baths have been described, for example, in U.S. Patents 2,748,000, May 29, 1956; 2,113,329, April 5, 1938; and 2,252,718, August 19, 1941.

Photographic silver halide emulsions useful in the process of the present invention can be prepared according to known methods such as those described in Hewittson and McClintock, U.S. Patent 2,618,556, November 18, 1952. Emulsions prepared by other methods can also be used to equal advantage in the invention. These emulsions can be sensitized, for example, with chemical sensitizers as described in U.S. Patents 2,540,085; 2,597,856; and 2,597,915; with azaindene compounds as disclosed in U.S. Patent 2,716,062; with condensation products of alkylene oxides as described in U.S. Patent 2,400,532; and with the additives as mentioned in U.S. Patent 2,937,089. In short, the photographic emulsions of the invention can contain addenda or not, as well known in the art, to improve the character of such emulsions.

Photographic elements of the present invention can be prepared by employing any of the emulsions previously described. Emulsions of the present type can be coated as separate layers on typical supports as used in preparing such photographic elements, such as cellulose acetate film, resin film, paper etc. Typical photographic elements of the invention which contain separate layers and are therefore referred to as multilayer materials have been described in such U.S. Patents as 1,055,155, March 4, 1913; 2,304,940, December 15, 1942; and 2,322,027, June 15, 1943.

The present invention is also applicable to color photographic emulsion materials wherein the emulsions are mixed instead of disposed in separate layers. Moreover, particular emulsions can be employed in the invention which comprise single emulsions containing color formers for making component color pictures. The emulsions of the present invention, in addition to containing color formers (couplers) as previously indicated, can also contain sensitizing dyes in addition to the usual addenda employed in emulsions of the present type.

The emulsions of the present photographic elements normally contain sensitizing dyes which render such emulsions more sensitive to particular regions of the spectrum. Such sensitization is normally referred to as optical sensitization and is well known in the art and has been described in such U.S. Patents as 2,640,776, June 2, 1953.

Our invention is especially useful where the emulsions contain, in addition to a color-former, a dispersing agent for the color-former, e.g., the water-insoluble but water-permeable materials set forth in U.S. Patents 2,304,940 and 2,322,027, such as water-insoluble but water-permeable cellulose esters, e.g., water-insoluble, but water-permeable cellulose acetate, cellulose acetate-phthalate,

cellulose nitrate, etc., water-insoluble, but water-permeable cellulose ethers, water-insoluble but water-permeable natural and synthetic resins, high-boiling, substantially water-insoluble crystalloidal materials, such as N-n-amyl-phthalimide, tetrahydrofurfuryl benzoate, triphenyl phosphate, n-butyl phthalate, and the like (see also U.S. 2,801,717).

Our invention is especially useful with emulsions in which the color-former is dispersed in one or more of the aforesaid substantially water-insoluble, high-boiling crystalloidal materials. These crystalloidal materials are organic and have boiling points above about 175° C. These crystalloidal materials have a high solvent action for the color-formers and for the dyes formed therefrom and are permeable to photographic processing solutions. These crystalloidal materials have been referred to as "oil formers" because they have the property of producing an oily or liquid solution when mixed with the coupler, even though the coupler is a solid. The crystalloidal materials are generally liquid at ordinary temperatures or low melting solids (below 100° C.). The most useful compounds contain one or more polar groups such as halogen, hydroxyl, carboxylic acid, amide, ketone, etc.

The following couplers are suitable for use in our invention. It is to be understood that this list is not exhaustive, but merely to typify compounds which may be used.

#### COUPLERS PRODUCING CYAN IMAGES

- 5-(p-amylphenoxybenzenesulfonamino)-1-naphthol  
 5-(N-benzyl-N-naphthalenesulfonamino)-1-naphthol  
 5-(n-benzyl-N-n-valerylamino)-1-naphthol  
 5-caproylamino-1-naphthol  
 2-chloro-5-(N-n-valeryl-N-p-isopropylbenzylamino)-1-naphthol  
 35 2,4-dichloro-5-(p-nitrobenzoyl-β-o-hydroxyethylamino)-1-naphthol  
 2,4-dichloro-5-palmithylamino-1-naphthol  
 2,2'-dihydroxy-5,5'-dibromostilbene  
 5-diphenylethersulfonamido-1-naphthol  
 40 1-hydroxy-2-(N-isoamyl-N-phenyl)naphthamide  
 1-hydroxy-2-(N-p-sec. amylphenyl)-naphthamide  
 8-hydroxy-1-α-naphthoyl-1,2,3,4-tetrahydroquinoline  
 2-lauryl-4-chlorophenol  
 1-naphthol-2-carboxylic-α-naphthalide  
 1-naphthol-5-sulfocyclohexylamide  
 5-phenoxyacetamino-1-naphthol  
 5-β-phenylpropionylamino-1-naphthol  
 Monochlor-5-(N-γ-phenylpropyl-N-p-sec.-amylbenzoyl-amino)-1-naphthol  
 2-acetylamino-5-methylphenol  
 50 2-benzoylamino-3,5-dimethylphenol  
 2-α-(p-tert. amylphenoxy)-n-butylamino-5-methyl-phenol

Any of the acylaminophenol couplers disclosed in United States Patents 2,423,730, dated July 8, 1947, can also be used as couplers for the cyan image.

#### COUPLERS PRODUCING MAGENTA IMAGES

- 1-p-sec. amylphenyl-3-n-amyl-5-pyrazolone  
 60 2-cyanoacetyl-5-(p-sec. amylbenzoyl-amino)-coumarone  
 2-cyanoacetylcoumarone-5-(N-n-amyl-p-tert. amylsulf-anilide)  
 2-cyanoacetylcoumarone-5-sulfon-N-n-butylanilide  
 2-cyanoacetyl-5-benzoylamino-coumarone  
 65 2-cyanoacetylcoumarone-5-sulfondimethylamide  
 2-cyanoacetylcoumarone-5-sulfon-N-methylanilide  
 2-cyanoacetylcoumarone-5-(N-γ-phenylpropyl)-p-tert. amylsulfonanilide  
 1-p-laurylphenyl-3-methyl-5-pyrazolone  
 70 1-β-naphthyl-3-amyl-5-pyrazolone  
 1-p-nitrophenyl-3-n-amyl-5-pyrazolone  
 1-p-phenoxyphenyl-3-n-amyl-5-pyrazolone  
 1-phenyl-3-n-amyl-5-pyrazolone  
 1,4-phenylene bis-3-(1-phenyl-5-pyrazolone)  
 75 1-phenyl-3-acetyl-amino-5-pyrazolone

## COUPLERS PRODUCING YELLOW IMAGES

- N-amyl-p-benzoylacetaminobenzenesulfonate  
 N-(4-anisoylacetaminobenzenesulfonyl)-N-benzyl-m-toluidine  
 N-(4-benzoylacetaminobenzenesulfonyl)-N-benzyl-m-toluidine  
 N-(4-benzoylacetaminobenzenesulfonyl)-N-n-amyl-p-toluidine  
 N-(4-benzoylacetaminobenzenesulfonyl)-N-benzylaniline  
 $\omega$ -(p-Benzoylbenzoyl)acetanilide  
 $\omega$ -Benzoylacet-2,5-dichloroanilide  
 $\omega$ -Benzoyl-p-sec. amylacetanilide  
 N,N'-di( $\omega$ -benzoylacetyl)-p-phenylenediamine  
 N,N'-di(acetoacetamino)diphenyl  
 4,4'-di(acetoacetamino)-3,3'-dimethylidiphenyl  
 p,p'-Di-(acetoacetamino)diphenylmethane  
 Ethyl-p-benzoylacetaminobenzenesulfonate  
 Nonyl-p-benzoylacetaminobenzenesulfonate  
 N-phenyl-N'-(p-acetoacetaminophenyl)-urea

In the development of exposed photographic silver halide emulsion layers using the couplers of our invention, any color-forming developer containing a primary amino group may be used. These include developers having two primary amino groups as well as those having one of the amino groups substituted or having substituents in the ring, such as the alkyl phenylene diamines. These compounds are usually used in the salt form, such as the hydrochloride or the sulfate which are more stable than the amines themselves. The suitable compounds are diethyl-p-phenylenediamine hydrochloride, monomethyl-p-phenylenediamine hydrochloride, dimethyl-p-phenylenediamine hydrochloride, and 2-amino-5-diethylaminotoluene hydrochloride. The p-amino phenols and their substitution products may also be used where the amino group is unsubstituted. All of these developers have an unsubstituted amino group which enables the oxidation products of the developer to couple with the color-forming compounds to form a dye image.

The color-formers (couplers) can be incorporated in the emulsions in the customary manner, e.g., by adding a dispersion of the coupler in a water-insoluble but water-permeable material to the emulsion as indicated previously, or by adding a dispersion of the alkali metal of the coupler in water. Couplers can also be added to the emulsion in crystalloidal materials such as oil-boiling organic crystalloidal materials to produce an oil-like mixture which can then be dispersed in water or a binder of colloidal character as well known in the art. (See for example U.S. Patent 2,640,776.) Dispersion of the coupler in a binder can be effected with the aid of a homogenizer, a colloid mill, or the like; and dispersions can be stabilized by the addition of emulsifying agents also well known in the art.

Sensitizing dyes of the type previously indicated normally are added to the emulsion before the coupler or coupler dispersion is added. (See for example U.S. Patent 2,640,776 and 2,407,210.) Typical sensitizing dyes for use in emulsions of the invention have been described in a number of U.S. and foreign patents, for example, U.S. Patents 2,478,366, August 9, 1949; 2,213,238, September 3, 1940; 2,231,658, February 11, 1941; and 2,515,913, July 18, 1950.

To further describe the invention, reference will now be made to the following examples.

## EXAMPLE I

A multilayer photographic element of the type described in Jelley and Vittum U.S. Patent 2,322,027, issued June 15, 1943, was used as the multilayer sensitive element. Separate elements of the type described were given a like exposure to a colored image in the usual manner and processed according to the following procedures in which one of said elements was processed in a

conventional manner (Process A) and the second element was processed according to the present invention (Process B).

## Process A (70° F.)

|    |               | Time            |
|----|---------------|-----------------|
| 5  | Color develop | 7 min. 30 sec.  |
|    | Wash          | 15 sec.         |
|    | Fix           | 4 min.          |
|    | Wash          | 4 min.          |
| 10 | Bleach        | 8 min.          |
|    | Wash          | 4 min.          |
|    | Fix           | 4 min.          |
|    | Wash          | 7 min.          |
| 15 | Buffer        | 1 min.          |
|    | Wash          | 2 sec.          |
|    | Total time    | 39 min. 47 sec. |

## Process B (70° F.)

|    |               | Time            |
|----|---------------|-----------------|
| 20 | Color develop | 7 min. 30 sec.  |
|    | Wash          | 15 sec.         |
|    | Acid stop     | 2 min.          |
|    | Bleach-fix    | 4 min.          |
| 25 | Bleach        | 4 min.          |
|    | Wash          | 7 min.          |
|    | Buffer        | 1 min.          |
|    | Wash          | 2 sec.          |
|    | Total Time    | 25 min. 47 sec. |

The processing solutions had the following formulations:

## COLOR DEVELOPER

|    |                                                                                                              |    |       |
|----|--------------------------------------------------------------------------------------------------------------|----|-------|
| 35 | Water                                                                                                        | ml | 950.0 |
|    | Benzyl alcohol                                                                                               | ml | 3.8   |
|    | Sodium sulfite                                                                                               | g  | 2.1   |
|    | Sodium hydroxide                                                                                             | g  | 0.45  |
| 40 | 4 - amino - N - ethyl - N - ( $\beta$ -methanesulfonamidoethyl) - meta - toluidine sesquisulfate monohydrate | g  | 5.0   |
|    | Sodium bromide                                                                                               | g  | 0.86  |
|    | Sodium carbonate (anhydrous)                                                                                 | g  | 42.7  |
|    | Water to make 1.0 liter.                                                                                     |    |       |
| 45 | pH 10.75 at 70° F.                                                                                           |    |       |

## FIX BATH

|    |                          |    |       |
|----|--------------------------|----|-------|
| 50 | Water                    | ml | 600.0 |
|    | Sodium thiosulfate       | g  | 240.0 |
|    | Sodium sulfite           | g  | 15.0  |
|    | Glacial acetic acid      | g  | 13.4  |
|    | Boric acid               | g  | 7.5   |
|    | Potassium alum           | g  | 15.0  |
|    | Water to make 1.0 liter. |    |       |
| 55 | pH 4.2 at 70° F.         |    |       |

## BLEACH BATH

|    |                        |    |       |
|----|------------------------|----|-------|
| 60 | Water                  | ml | 800.0 |
|    | Potassium ferricyanide | g  | 50.0  |
|    | Potassium bromide      | g  | 20.0  |

|    |                          |  |  |
|----|--------------------------|--|--|
| 65 | Water to make 1.0 liter. |  |  |
|    | pH 6.5 at 70° F.         |  |  |

## BUFFER BATH

|    |                             |    |       |
|----|-----------------------------|----|-------|
| 70 | Water                       | ml | 800.0 |
|    | Disodium hydrogen phosphate | g  | 8.2   |
|    | Glacial acetic acid         | ml | 4.5   |
|    | Water to make 1.0 liter.    |    |       |

## ACID STOP BATH

|    |                                                                                  |    |       |
|----|----------------------------------------------------------------------------------|----|-------|
| 75 | Water                                                                            | ml | 600.0 |
|    | Sodium sulfite                                                                   | g  | 15.0  |
|    | Glacial acetic acid                                                              | ml | 15.0  |
|    | Water to make 1.0 liter.                                                         |    |       |
|    | Adjustment to final pH of 4.2 using acetic acid or sodium hydroxide as required. |    |       |

7  
BLEACH-FIX BATH

|                                                   | G.    |
|---------------------------------------------------|-------|
| Ferric chloride (6H <sub>2</sub> O)               | 24.0  |
| Ethylenediamine tetraacetic acid tetrasodium salt | 40.0  |
| Sodium thiosulfate (5H <sub>2</sub> O)            | 150.0 |
| Sodium sulfite                                    | 15.0  |
| pH 7.0 at 70° F.                                  |       |

In either of the processes of the example, color development formed silver, cyan magenta, and yellow dye densities in the sensitive layers of the element; and after development in each process, the emulsion layers were cleared of silver and silver halides, leaving the respective dye densities in situ.

Process A, a conventional process, required 39 minutes, 47 seconds and employed ten steps including development, whereas processing according to the present invention (Process B) required 25 minutes, 47 seconds and employed eight steps. The process of the present invention, in effect, reverses the normal processing order by employing a bleach bath subsequent to a fixing bath to clear the photographic material of silver and silver halide from the emulsion layers.

The sensitometric results of the example are shown in the accompanying drawing in which FIG. 1 shows the sensitometric curves obtained from the material processed according to Process A and FIG. 2 shows the sensitometric curves obtained in a comparable element processed according to Process B.

More particularly, in FIG. 1, sensitometric curve 10 shows the integral cyan dye density of the processed element as measured in a well known manner on an Eastman Electronic densitometer using a tungsten light source and red-light transmitting filter. Sensitometric curves 11 and 12 show the integral magenta and yellow dye densities, respectively, as measured in like manner using a green-light transmitting filter for the magenta dye density determination and a blue-light transmitting filter for the yellow dye density determination.

In FIG. 2, sensitometric curves 13, 14, and 15 show, respectively, the cyan, magenta and yellow integral dye densities obtained in like manner in the element processed according to Process B. The density measurements were made employing, respectively, red-, green- and blue-light transmitting sources as in the FIG. 1 determination.

The retention of silver in the elements processed in the present example was in each case 1 mg. or less per square foot for the elements processed according to either of Processes A or B as determined in a well known manner, for example, by X-ray fluorescence analysis. The elements used in the present example contained in excess of 200 mg. of silver per square foot prior to processing.

## EXAMPLE II

Separate multilayer photographic elements of the type used in Example I were exposed to a multicolored image in a well known manner after which one strip was processed according to a conventional process (Process C) and the second strip was processed according to the process of the present invention (Process D).

## Process C

|                   | Min. |
|-------------------|------|
| Color develop     | 12   |
| Stop bath         | 2    |
| First fix         | 2    |
| Wash              | 2    |
| Bleach            | 4    |
| Wash              | 2    |
| Hardener fix      | 2    |
| Wash              | 8    |
| Formalin hardener | 3    |
| Wash              | 3    |
| Buffer            | 3    |
| Total time        | 43   |

8  
Process D

|                    | Min. |
|--------------------|------|
| Color develop      | 12   |
| Acid-hardener bath | 2    |
| 5 Bleach-fix       | 2    |
| Bleach             | 4    |
| Wash               | 8    |
| Buffer             | 3    |
| Total time         | 29   |

The processing solutions not previously disclosed had the following formulations:

## COLOR DEVELOPER

|    |                                                                                                        |    |      |
|----|--------------------------------------------------------------------------------------------------------|----|------|
| 15 | Benzyl alcohol                                                                                         | ml | 12.6 |
|    | Sodium hexametaphosphate                                                                               | g  | 2.0  |
|    | Sodium sulfite                                                                                         | g  | 2.1  |
| 20 | Sodium carbonate                                                                                       | g  | 26.8 |
|    | Potassium bromide                                                                                      | g  | 0.48 |
|    | Sodium chloride                                                                                        | g  | 0.70 |
|    | Hydroxylamine sulfate                                                                                  | g  | 2.1  |
| 25 | 4 - amino - N - ethyl - N-( $\beta$ -methanesulfonamidoethyl)-meta-toluidine sesquisulfate monohydrate | g  | 4.2  |
|    | Water to 1.0 liter.                                                                                    |    |      |
|    | pH 9.96 at 75° F.                                                                                      |    |      |

## STOP BATH

|    |                     |    |      |
|----|---------------------|----|------|
| 30 | Glacial acetic acid | ml | 17.0 |
|    | Sodium sulfite      | g  | 20.0 |
|    | Water to 1.0 liter. |    |      |
|    | pH 4.64 at 75° F.   |    |      |

## FIRST FIXING BATH

|    |                             |   |       |
|----|-----------------------------|---|-------|
| 35 | Boric acid                  | g | 5.0   |
|    | Potassium alum              | g | 24.0  |
|    | Sodium thiosulfate          | g | 223.0 |
| 40 | Sodium bisulfite            | g | 12.0  |
|    | Sodium acetate (desiccated) | g | 14.0  |
|    | Sodium citrate (desiccated) | g | 1.7   |
|    | Water to 1.0 liter.         |   |       |
|    | pH 4.40 at 75° F.           |   |       |

## BLEACH BATH

|    |                        |   |      |
|----|------------------------|---|------|
| 45 | Sodium nitrate         | g | 45.0 |
|    | Potassium ferricyanide | g | 22.5 |
| 50 | Potassium bromide      | g | 8.2  |
|    | Boric acid             | g | 7.5  |
|    | Borax                  | g | 0.97 |
|    | Water to 1.0 liter.    |   |      |
|    | pH 7.30 at 75° F.      |   |      |

## HARDENER-FIX BATH

|    |                     |   |       |
|----|---------------------|---|-------|
| 55 | Glacial acetic acid | g | 15.0  |
|    | Zinc sulfate        | g | 7.5   |
| 60 | Sodium citrate      | g | 2.5   |
|    | Zircotan            | g | 0.46  |
|    | Sodium bisulfite    | g | 17.9  |
|    | Boric acid          | g | 7.2   |
| 65 | Potassium alum      | g | 35.5  |
|    | Sodium thiosulfate  | g | 167.7 |
|    | Water to 1.0 liter. |   |       |
|    | pH 4.40 at 75° F.   |   |       |

## FORMALIN-HARDENER BATH

|    |                                   |    |      |
|----|-----------------------------------|----|------|
| 70 | Calgon (sodium hexametaphosphate) | g  | 0.75 |
|    | Sodium carbonate                  | g  | 8.8  |
|    | Formaldehyde (37% solution)       | ml | 25.5 |
|    | Water to 1.0 liter.               |    |      |

43 75 pH 10.90 at 75° F.

## BUFFER BATH

|                         |     |      |
|-------------------------|-----|------|
| Citric acid             | g.  | 30.0 |
| Borax                   | g.  | 20.4 |
| Formalin (37% solution) | ml. | 17.0 |
| Zinc sulfate            | g.  | 10.0 |
| Water to 1.0 liter.     |     |      |
| pH 3.5 at 75° F.        |     |      |

## ACID-HARDENER BATH

|                     |     |       |
|---------------------|-----|-------|
| Water               | ml. | 600.0 |
| Sodium sulfite      | g.  | 15.0  |
| Glacial acetic acid | g.  | 13.4  |
| Boric acid          | g.  | 7.5   |
| Potassium alum      | g.  | 15.0  |
| Water to 1.0 liter. |     |       |

## BLEACH-FIX BATH

|                                        |    |       |
|----------------------------------------|----|-------|
| Ferric chloride (6H <sub>2</sub> O)    | G. | 24.0  |
| Ethylenediamine tetraacetic acid       |    | 40.0  |
| Sodium thiosulfate (5H <sub>2</sub> O) |    | 150.0 |
| Thiourea                               |    | 5.0   |
| Sodium sulfite                         |    | 15.0  |
| Water to 1.0 liter.                    |    |       |
| pH 7.0 at 70° F.                       |    |       |

The processing time for the standard process (Process C) of the example was 43 minutes as compared to a 29-minute process time for Process D. Substantially the same sensitometric results and silver retention were obtained in either case. Each element contained an excess of 200 mg. of silver per square foot prior to processing.

## EXAMPLE III

Separate strips of a photographic material of the type described in Jolley et al. U.S. Patent 2,322,027 coated on a paper support were exposed to a multicolored positive transparency in the usual manner and processed separately according to the following procedures, in which Process E is a standard reversal process and Process F is a reversal process of the present invention.

## Process E

|                       |  |                 |
|-----------------------|--|-----------------|
| Presoak               |  | 2 min.          |
| Drain                 |  | 2 min.          |
| First developer       |  | 6 min.          |
| First stop            |  | 3 min.          |
| Wash                  |  | 7 min. 15 sec.  |
| Reversal exposure:    |  |                 |
| Color develop         |  | 7 min. 15 sec.  |
| Second stop           |  | 3 min.          |
| Wash                  |  | 7 min. 15 sec.  |
| Bleach                |  | 7 min. 15 sec.  |
| Wash                  |  | 7 min. 15 sec.  |
| Hardener-fix          |  | 7 min. 15 sec.  |
| Wash                  |  | 14 min. 30 sec. |
| Stabilizer            |  | 1 min.          |
| Total processing time |  | 75 min.         |

## Process F

|                       |  |                 |
|-----------------------|--|-----------------|
| Presoak               |  | 2 min.          |
| Drain                 |  | 2 min.          |
| First developer       |  | 6 min.          |
| First stop            |  | 3 min.          |
| Wash                  |  | 7 min. 15 sec.  |
| Reversal exposure:    |  |                 |
| Color develop         |  | 7 min. 15 sec.  |
| Second stop           |  | 3 min.          |
| Bleach-fix            |  | 4 min.          |
| Bleach                |  | 4 min.          |
| Wash                  |  | 14 min. 30 sec. |
| Stabilizer            |  | 1 min.          |
| Total processing time |  | 54 min.         |

Processing solutions used in the present example which have not been previously disclosed herein had the following formulations:

## FIRST DEVELOPER

|    |                                              |     |      |
|----|----------------------------------------------|-----|------|
| 5  | N-methyl-p-aminophenol sulfate               | g.  | 0.9  |
|    | Sodium sulfite                               | g.  | 8.0  |
|    | Hydroquinone                                 | g.  | 2.35 |
|    | Potassium bromide                            | g.  | 0.55 |
|    | Sodium metaborate (8H <sub>2</sub> O)        | g.  | 25.5 |
| 10 | 6-nitrobenzimidazole nitrate (0.5% solution) | ml. | 12.0 |
|    | Water to 1.0 liter.                          |     |      |
|    | pH 10.03 at 75° F.                           |     |      |

## FIRST STOP BATH

|    |                                                                         |     |      |
|----|-------------------------------------------------------------------------|-----|------|
| 15 | Sodium acetate                                                          | G.  | 3.0  |
|    | Glacial acetic acid                                                     |     | 19.0 |
|    | Water to 1.0 liter.                                                     |     |      |
|    | (Adjust to pH 3.7 at 75° F. using sodium hydroxide.)                    |     |      |
| 20 | Potassium iodide                                                        | g.  | 0.2  |
|    | Sodium bisulfite                                                        | g.  | 15.0 |
|    | Glacial acetic acid                                                     | ml. | 20.0 |
|    | Potassium alum                                                          | g.  | 30.0 |
| 25 | (Adjust to pH 3.0 using sodium hydroxide or sulfuric acid as required.) |     |      |

## BLEACH BATH

|    |                        |    |      |
|----|------------------------|----|------|
| 30 | Sodium nitrate         | G. | 30.0 |
|    | Potassium ferricyanide |    | 30.0 |
|    | Potassium bromide      |    | 15.0 |
|    | Borax                  |    | 1.0  |
|    | Boric acid             |    | 15.0 |
|    | Water to 1.0 liter.    |    |      |
| 35 | pH 6.7 at 75° F.       |    |      |

## HARDENER-FIX

|    |                     |    |       |
|----|---------------------|----|-------|
| 40 | Boric acid          | G. | 50.0  |
|    | Sodium thiosulfate  |    | 225.0 |
|    | Sodium bisulfite    |    | 10.0  |
|    | Sodium acetate      |    | 15.0  |
|    | Potassium alum      |    | 20.0  |
|    | Sodium citrate      |    | 2.0   |
|    | Water to 1.0 liter. |    |       |
| 45 | pH 4.6 at 75° F.    |    |       |

## STABILIZER

|    |                         |       |      |
|----|-------------------------|-------|------|
| 50 | Formalin (37% solution) | ml.   | 10.0 |
|    | Water to                | liter | 1.0  |

The process time in the present example was shortened from 75 minutes to 54 minutes and resulted in reduced stain density according to the following data.

|                         | Stain Density | Red | Green | Blue |
|-------------------------|---------------|-----|-------|------|
| Process E               |               | 22  | 22    | 26   |
| Process F               |               | 18  | 17    | 18   |
| Change in stain density |               | 4   | 5     | 9    |

The stain densities were measured in a well known manner by reflection densitometry in which the integral dye densities in the cyan, magenta, and yellow were determined using red-, green- and blue-transmitting filters, respectively.

In the present process, good image densities are obtained presumably since the invention permits the use of a final bleach which oxidizes leuco dye present to full color intensity. The photographic materials of the previous examples contained in excess of 200 mg. of silver per square foot. The silver retained after processing

70 was equal to or less than the silver retention in conventionally processed elements which involved more time and a greater number of steps. Photographic materials having from 200 to about 600 mg. of silver per square foot can be processed to an optimum photographic result by way of the present invention.

The invention has been described in detail with particular reference to preferred embodiments thereof but it will be understood that variations and modifications can be effected within the spirit and scope of the invention as described hereinabove and as defined in the appended claims.

We claim:

1. In the color processing of an exposed photographic silver halide emulsion layer containing a color coupler that has been color developed to form a dye image, the improvement which comprises treating the said color developed emulsion layer with an aqueous solution containing ferric chloride and a thiosulfate silver halide solvent and thereby solubilizing and removing silver and silver halide from said emulsion layer, and thereafter further treating the resulting emulsion layer with an aqueous solution containing a ferricyanide silver oxidizing agent and thereby oxidizing leuco dye in said emulsion layer to full color intensity.

2. In the color processing of an exposed photographic silver halide emulsion layer containing a color coupler that has been color developed to form a dye image, the improvement which comprises treating the said color developed emulsion layer with an aqueous solution containing ferric chloride and an alkali metal thiosulfate and thereby solubilizing and removing silver and silver halide from said emulsion layer, and thereafter further treating the resulting emulsion layer with an aqueous solution containing an alkali metal ferricyanide and thereby oxidizing leuco dye in said emulsion layer to the full color intensity of the dye.

3. In the color processing of an exposed photographic silver halide emulsion layer containing a color coupler that has been color developed to form a dye image, the improvement which comprises treating the said color developed emulsion layer with an aqueous solution containing ferric chloride, ethylenediamine tetraacetic acid, sodium thiosulfate and sodium sulfite and thereby solubilizing and removing silver and silver halide from said emulsion layer, and thereafter further treating the resulting emulsion layer with an aqueous solution containing potassium ferricyanide and thereby oxidizing leuco dye in said emulsion layer to full color intensity.

4. The process as described in claim 1 wherein the silver halide emulsion layer contains in excess of 200 mg. of silver per square foot.

#### References Cited by the Examiner

##### UNITED STATES PATENTS

|           |      |                    |       |
|-----------|------|--------------------|-------|
| 2,380,809 | 7/45 | Verkinderen et al. | 96—55 |
| 2,506,622 | 5/50 | Tull               | 96—55 |
| 2,737,457 | 3/56 | Childress          | 96—55 |
| 2,752,244 | 6/56 | Sprung             | 96—22 |

##### FOREIGN PATENTS

|           |      |          |
|-----------|------|----------|
| 1,051,117 | 2/59 | Germany. |
|-----------|------|----------|

NORMAN G. TORCHIN, Primary Examiner.

LOUISE P. QUAST, Examiner.